

## UNITED STATES PATENT OFFICE

2,663,691

## GREASE CONTAINING DIPHENYL P-PHENYLENE DIAMINE AND A PHOSPHORUS ACID ESTER AND METHOD OF MAKING SAID GREASE

John P. Dilworth, Fishkill, N. Y., assignor to The Texas Company, New York, N. Y., a corporation of Delaware

No Drawing. Application February 16, 1951,  
Serial No. 211,447

12 Claims. (Cl. 252—42.1)

1

The present invention relates to lubricating compositions and to a method of making them. More particularly it relates to lubricating greases containing a small amount of N,N' diphenyl para-phenylene diamine associated with an oil-soluble phosphorus acid ester as a carrier.

It has been proposed heretofore to employ N,N' diphenyl para-phenylene diamine as an anti-oxidant in organic compositions normally subject to oxidative deterioration such as rubber, gasoline and lubricating compositions. The pending co-owned application of George W. Eckert, Serial No. 211,446, filed of even date herewith, discloses and claims that this compound has important advantages over other amines commonly employed as oxidation inhibitors, including closely analogous derivatives of para-phenylene diamine, when employed in a sodium myristate type of ball and roller bearing grease, by imparting unexpectedly superior thermal stability to the grease when used for the lubrication of anti-friction bearings at high temperatures of the order of 300° F.

However, difficulties have been encountered in the uniform incorporation of N,N' diphenyl para-phenylene diamine into such lubricating grease compositions because of its insolubility in the high boiling organic liquid lubricating bases which normally comprise a major portion of such compositions. When this compound is incorporated into greases by the usual methods employed with insoluble or difficultly soluble additives, such as by heating the lubricant base to a temperature above the melting point of the additive compound or by adding the latter to the lubricant base or grease in solution in a light organic solvent, which is later flashed off, non-uniform lubricating grease compositions may be produced having widely varying thermal stability characteristics, and the N,N' diphenyl para-phenylene diamine shows a tendency to crystallize out of the grease upon cooling.

It is accordingly a principal object of the present invention to provide an improved grease composition, and a method of manufacturing such composition, containing N,N' diphenyl para-phenylene diamine, whereby a uniform composition having superior thermal stability and other advantages is obtained.

In accordance with the present invention, this is accomplished by adding to such lubricating grease compositions a minor amount of N,N' diphenyl para-phenylene diamine dissolved in an oil-soluble ester of a phosphorus acid. Phosphorus acid esters which are particularly suitable

for this purpose are tri-alkyl, aryl and mixed alkyl-aryl esters of phosphoric and phosphorous acids boiling above about 400° F. As examples of such compounds may be mentioned tributyl phosphate, triamyl phosphate, tricresyl phosphate, tricresyl phosphite, trixylyl phosphate and trixylyl phosphite. Tricresyl phosphate, obtained from coal tar acids, is an especially suitable and readily available material of this type. The phosphorus acid ester serves as a carrier and a distributor for the N,N' diphenyl para-phenylene diamine so that the latter can be readily incorporated into the grease, forming a uniform and stable composition. Furthermore, it has been found that a synergistic effect of the phosphorus acid ester and the amine is thus obtained on the thermal stability of the grease composition, while in addition known anti-wear properties of the phosphorus acid ester are imparted to the grease.

20 A suitable inhibitor composition of my invention comprises tricresyl phosphate containing dissolved therein N,N' diphenyl para-phenylene diamine in at least a 2.5:1 weight ratio and up to about 20:1 or higher depending upon the permissible amount of tricresyl phosphate which may be added to the grease, and preferably about a 2.7:1 to 4:1 weight ratio. Such a solution may be obtained by dissolving N,N' diphenyl para-phenylene diamine in tricresyl phosphate when the latter is heated at about 200° F. At this temperature tricresyl phosphate dissolves a little over one third of its weight of N,N' diphenyl para-phenylene diamine.

35 A solution of N,N' diphenyl para-phenylene diamine in an oil-soluble phosphorus acid ester obtained in the above described manner, or in any other suitable manner, is added to lubricating grease compositions in amounts sufficient to impart the desired thermal stability, oxidation resistance and anti-wear properties to the latter. Generally, the solution is added in an amount such that the lubricating composition contains from about 0.1 per cent to about 8 per cent, and preferably from about 0.5 per cent to about 2 per cent by weight of N,N' diphenyl para-phenylene diamine.

40 Lubricating grease compositions to which the inhibitor composition of my invention may be added suitably comprise in substantial proportion a high boiling organic oil, which may be a mineral oil fraction obtained from a paraffinic, naphthenic or mixed base crude by any of the usual refining methods, an animal or vegetable oil such as lard oil, corn oil, castor oil, or the like, or a 45 synthetic oil obtained by polymerization or

50 55

chemical condensation, as well as mixtures of these. The lubricating compositions may contain any of the usual additives in so far as no incompatibility exists between them and the additives of my invention, as well as thickening agents such as fatty acid soaps in grease forming proportions.

An especially valuable embodiment of my invention comprises imparting superior thermal stability to a sodium base ball and roller bearing grease prepared from a mixture of low molecular weight fatty acids comprising at least 70 per cent, and preferably at least 90 per cent, of myristic acid and/or the glycerides thereof. The grease preferably comprises from about 15 per cent to about 25 per cent of a soap obtained by saponifying such a fatty acid mixture with a small excess of alkali, and a lubricating oil which may suitably be a blend of a distillate oil and a residual oil from a paraffinic stock. Greases of this type are particularly useful as lubricants for ball and roller bearings operated at high rotative speeds and under elevated temperatures up to 300° F. and above.

The table below gives data obtained on several greases of the above type containing N,N'-diphenyl para-phenylene diamine as the oxidation inhibitor which was added both by the conventional methods and by the method of my invention. Comparative data are also included on an uninhibited grease of this type and on such

temperature was maintained at 295-320° F. for two and one half hours to effect dehydration while the stirring was continued, and the temperature then allowed to decrease gradually while the remainder of the mineral oil was added. The temperature reduction was controlled during the oil addition so that a total amount of mineral oil equal to at least twice the weight of the fatty acid was charged before the temperature was allowed to drop below 260° F.

In the preparation of Grease #3 of the table, N,N'-diphenyl para-phenylene diamine was dissolved in a mixture of benzene and acetone and added to a portion of the base oil at 250° F. The mixture was then heated for four hours to drive off the solvent and the remaining composition added to the grease at the end of the manufacturing process. In the preparation of Grease #4, the N,N'-diphenyl para-phenylene diamine was added to the grease in the form of a slurry in a part of the residual base oil at the end of the manufacturing process. In the case of Greases #5, #6 and #7, the N,N'-diphenyl para-phenylene diamine was dissolved in tricresyl phosphate at about 200° F. and the resulting solution added to the grease at the end of the manufacturing process while the grease was at a temperature of about 200° F. The additive solution is generally stirred into the grease following dehydration and after the temperature of the grease has dropped below 250° F.

TABLE

|                                                                               | No. 1 | No. 2 | No. 3                      | No. 4                   | No. 5                                             | No. 6 | No. 7 |
|-------------------------------------------------------------------------------|-------|-------|----------------------------|-------------------------|---------------------------------------------------|-------|-------|
| Grease composition, percent:                                                  |       |       |                            |                         |                                                   |       |       |
| Na myristate                                                                  | 15.7  | 20.0  | 19.8                       | 20.0                    | 15.1                                              | 16.4  | 13.1  |
| Distillate oil                                                                | 14.7  | 14.0  | 14.7                       | 14.0                    | 14.2                                              | 12.3  | 12.7  |
| Residual oil                                                                  | 69.2  | 60.5  | 60.0                       | 60.5                    | 66.6                                              | 67.1  | 70.1  |
| Excess NaOH                                                                   | 0.4   | 0.5   | 0.5                        | 0.5                     | 0.4                                               | 0.5   | 0.4   |
| Diphenylamine                                                                 | 0     | 5.0   |                            |                         |                                                   |       |       |
| DPD <sup>1</sup>                                                              | 0     |       | 5.0                        | 5.0                     | 1.0                                               | 1.0   | 1.0   |
| Tricresyl phosphate                                                           | 0     |       |                            |                         | 2.7                                               | 2.7   | 2.7   |
| Method of DPD <sup>1</sup> addition                                           |       |       | In benzene acetone solvent | In heavy oil at 300° F. | DPD <sup>1</sup> dissolved in tricresyl phosphate |       |       |
| Tests on product:                                                             |       |       |                            |                         |                                                   |       |       |
| Dropping point, ° F.                                                          | 432   | 457   | 423                        | 452                     | 431                                               | 404   | 406   |
| Unworked penetration                                                          | 222   | 191   | 176                        | 104                     | 223                                               | 198   | 240   |
| Worked penetration                                                            | 289   | 285   | 328                        | 208                     | 304                                               | 255   | 287   |
| Free NaOH, percent                                                            | 0.39  |       |                            | 0.27                    | 0.22                                              | 0.17  | 0.20  |
| Alkaline                                                                      |       |       |                            | 0                       | 0.04                                              | 0.03  | 0.04  |
| Free fatty acid, percent                                                      |       |       |                            |                         | 4                                                 | 5     | 3     |
| Norma-Hoffmann oxidation, pressure drop in 100 hours                          | 35    |       | 12                         |                         |                                                   |       |       |
| High temperature performance test (300° F., 10,000 R. P. M.) hours to failure | 389   | 352   | 368                        | 838                     | 807                                               | 1,308 | 744   |
|                                                                               | 280   |       | 627                        |                         |                                                   |       | 1,152 |
|                                                                               | 294   |       | 570                        | 430                     |                                                   |       |       |

<sup>1</sup> DPD is N,N'-diphenyl p-phenylene diamine.

a grease inhibited with an amine oxidation inhibitor of the usual type.

The greases were prepared by saponification of myristic acid with a slight excess of sodium hydroxide solution in the presence of a small amount of mineral oil and water, dehydrating the resulting soap base and adding sufficient mineral oil to obtain the desired consistency. The myristic acid employed had a saponification number of 245, a neutralization number of 242 and a titer of 45.7° C. The mineral oil was a blend comprising about 14 to 19 per cent of a solvent refined and clay treated paraffinic distillate oil having an SUS viscosity of 93 at 210° F. and the remainder a solvent refined, clay and acid treated paraffinic residual oil having an SUS viscosity of 120 at 210° F. The saponification was carried out by heating the charge consisting of myristic acid with about two thirds its weight of the distillate oil and a like amount of water to 170-190° F. and adding the sodium hydroxide solution with stirring. After the saponification the

55 foregoing table is a measure of the resistance to oxidation of lubricating greases when stored under static conditions for long periods of time, as when coated in thin films on anti-friction bearings, motor parts, etc. In this test, five four-60 gram samples of the grease are put in flat sample dishes and placed in a stainless steel bomb sealed with a lead gasket in an atmosphere of oxygen under an initial pressure of 110 pounds per square inch at a temperature of 210° F. The pressure 65 drop in pounds within the bomb is then recorded at intervals of 100 hours up to 400 hours or until a pressure drop of 55 pounds per square inch occurs.

The high temperature performance test is a 70 test for determining the performance characteristics of greases in anti-friction bearings at elevated temperatures and high rotative speeds. The test unit consists essentially of a steel spindle supported on ball bearings and driven by an electric motor connected into an electric circuit con-

taining a low amperage fuse 0.1 ampere below that required for full load running. The bearings are Norma-Hoffmann ABEC No. 3 grade and, are mounted on the spindle approximately 5% inches apart. A thrust load of 17.5 pounds is applied to these bearings. One of the bearings, which serves as the test bearing, is surrounded by an electrically heated housing. The other bearing is outside the heated chamber and serves only as a guide bearing. The test consists of operating the test bearing for twenty-four hours at 10,000 R. P. M. and 300° F., followed by a shut down and cooling period of two hours, and repeating this cycle until the lubricant fails, which is indicated by rupture of the low amperage fuse in the motor circuit. In starting up the test, three grams of the test grease are charged to the test bearing and worked into and around the races and balls. The test bearing is next rotated both clockwise and counter-clockwise for one minute each at 200 R. P. M. and assembled into the test unit. The heaters and the motor are then started and the test bearing brought up to the test temperature of 300° F. as rapidly as possible, which requires 1.0 to 1.25 hours, while the spindle is rotated at a speed of 10,000 R. P. M. After 24 hours of operation the heaters and motor are shut off for 2 hours, during which the temperature of the test bearing drops to a minimum of 120-130° F. The total hours of operation, excluding the two hour shut-down periods, to the failure point is recorded as the "hours to failure."

As shown in the foregoing table, greases having excellent thermal stability and other lubricating properties for high temperature ball and roller bearing service are produced by adding a minor proportion of N,N' diphenyl para-phenylene diamine dissolved in a small amount of tricresyl phosphate to sodium myristate base greases. The greases thus produced are markedly superior in these properties to greases of similar composition and manufacture having the inhibitor added according to the usual methods.

While the above examples serve to illustrate the results obtainable by the method of my invention, it is not intended to limit my invention to the manufacture of sodium myristate greases, since it is of general application to greases of various soap bases where highly effective oxidation resistance and/or thermal stability, in addition to anti-wear qualities, are desired. Thus it may be employed for improving lithium, calcium, barium or mixed base greases for various types of service.

Obviously many modifications and variations of the invention, as hereinbefore set forth, may be made without departing from the spirit and scope thereof, and therefore only such limitations should be imposed as are indicated in the appended claims.

I claim:

1. A lubricating grease composition comprising a lubricating oil, a metal soap of a fatty acid in grease forming proportion, a minor amount sufficient to impart thermal stability properties to the composition of N,N' diphenyl para-phenylene diamine added to the composition in solution in a minor amount of an oil-soluble phosphorus acid ester, the latter serving as a carrier and a dispersing agent for the N,N' diphenyl para-phenylene diamine.

2. Claim 1 wherein the phosphorus acid ester is tricresyl phosphate.

3. Claim 1 wherein the N,N' diphenyl para-

phenylene diamine comprises between about 0.1 per cent and about 8 per cent of the total weight of the lubricating composition.

4. Claim 1 wherein the metal soap is sodium myristate.

5. Claim 1 wherein the lubricating oil is a blend of a distillate and a residual oil of a paraffin base stock.

10 6. A lubricating grease consisting essentially of the following ingredients in the approximate specified proportions.

|                                      | Per cent |
|--------------------------------------|----------|
| Sodium myristate                     | 15-25    |
| N,N' diphenyl para-phenylene diamine | 0.5-5    |
| Tricresyl phosphate                  | 1.5-15   |
| Lubricating oil, remainder.          |          |

20 7. A lubricating grease consisting essentially of the following ingredients in the approximate specified proportions:

|                                                                                                             | Per cent |
|-------------------------------------------------------------------------------------------------------------|----------|
| Sodium myristate                                                                                            | 15-25    |
| N,N' diphenyl para-phenylene diamine                                                                        | 1        |
| Tricresyl phosphate                                                                                         | 2.7      |
| Excess NaOH                                                                                                 | 0.5      |
| Lubricating oil comprising a blend of a paraffinic distillate oil and a paraffinic residual oil, remainder. |          |

25 8. The method of improving the thermal stability of a lubricating grease composition consisting essentially of a lubricating oil and a fatty acid soap by adding thereto a small proportion of N,N' diphenyl para-phenylene diamine dissolved in tricresyl phosphate.

30 9. The method of manufacturing a ball and roller bearing grease adapted for high temperature lubrication of anti-friction bearings, which comprises saponifying a fatty material contain-

35 ing at least 70 per cent of a myristic acid with an excess of caustic soda in the presence of a small proportion of lubricating oil ultimately present in the grease, dehydrating the resulting saponified material by heating to 295-320° F., adding

40 additional lubricating oil to the dehydrated product as the temperature is lowered to obtain a grease of buttery consistency, and adding to the grease with stirring when the temperature has dropped below 250° F. a solution of N,N' diphenyl para-phenylene diamine in tricresyl phosphate in an amount effective to materially improve the thermal properties of the grease.

45 10. The method of manufacturing a ball and roller bearing grease adapted for high temperature lubrication of antifriction bearings, which comprises saponifying a fatty material contain-

50 ing at least 70 per cent myristic acid with a small excess of caustic soda in the presence of a small proportion of lubricating oil equal to about two thirds the weight of the fatty material and of a small amount of water approximately equal to the weight of the lubricating oil, then heating the saponification mass at 295-320° F. for at least

55 two hours to effect dehydration, then lowering the temperature of the mass gradually to 260° F. while an amount of lubricating oil is added sufficient to bring the total lubricating oil content of the mass to at least twice the weight of fatty material initially charged, then adding to the mass at a temperature below 260° F. additional lubricating oil sufficient to give a finished product having a soap content between about 15 per cent and about 25 per cent by weight, and adding to the mass at a temperature below about 250° F. a solution of N,N' diphenyl para-phenylene di-

amine in tricresyl phosphate in an amount effective to materially improve the thermal properties of the grease.

11. The method of improving the thermal stability of a lubricating grease composition consisting essentially of a lubricating oil and a fatty acid soap by adding thereto a small proportion of N,N' diphenyl para-phenylene diamine dissolved in an oil-soluble ester of a phosphorus acid.

12. A lubricating grease adapted for the high temperature lubrication of anti-friction bearings consisting essentially of the following ingredients in the approximate specified proportions:

|                                      | Per cent | 15 |
|--------------------------------------|----------|----|
| Sodium myristate                     | 15-25    |    |
| N,N' diphenyl para-phenylene diamine | 0.5-5    |    |
| Tricresyl phosphate                  | 1.5-15   |    |
| Lubricating oil, remainder.          |          |    |

said N,N' diphenyl para-phenylene diamine being uniformly dispersed through the grease by addition in solution in the said tricresyl phosphate.

JOHN P. DILWORTH.

References Cited in the file of this patent

UNITED STATES PATENTS

| Number    | Name            | Date           |
|-----------|-----------------|----------------|
| 2,229,030 | Adams           | Jan. 21, 1941  |
| 2,351,384 | Woods           | June 13, 1944  |
| 2,369,705 | Woodward et al. | Feb. 20, 1945  |
| 2,406,655 | Bax et al.      | Aug. 27, 1946  |
| 2,406,722 | Vincent         | Aug. 27, 1946  |
| 2,428,123 | Morgan et al.   | Sept. 30, 1947 |
| 2,542,570 | Puryear         | Feb. 20, 1951  |